

## UNITED STATES PATENT OFFICE

EDMUND A. ANDERSON, OF PALMERTON, PENNSYLVANIA, ASSIGNOR TO THE NEW JERSEY ZINC COMPANY, OF NEW YORK, N. Y., A CORPORATION OF NEW JERSEY

## ZINC BASE DIE-CASTING ALLOY

No Drawing.

Application filed June 5, 1929. Serial No. 368,730.

This invention relates to zinc base die-casting alloys and has for its object the provision of an improved alloy of this character. A further object of the invention is the provision of a die-casting made of a zinc base alloy and possessing improved and superior physical properties.

The mechanical requirements of the die-casting operation necessitate the construction 10 of the melting pot and die from iron and steel. These metals are subject to attack by molten zinc and it has been found from experience, to minimize this attack sufficiently to secure reasonable life from the machines, 15 that at least 0.25% aluminum must be added to the zinc. Alloys for die-casting must possess a sufficient degree of fluidity to properly flow into and completely fill the dies used, and 2% or more aluminum appears to 20 be necessary to secure an adequate degree of fluidity. It has also long been known that aluminum increases the tensile strength of zinc and this, in itself, makes its presence in zinc base die-casting alloys desirable in 25 quantities of from 2% to as much as 10 to 15%.

Zinc-aluminum alloys containing less than 30 about 80% of aluminum undergo a structural change subsequent to solidification which is commonly known as a phase change or more 35 specifically in this case as an eutectoid reaction. This phase change consists in the formation of two crystalline forms or phases from one phase previously existing, and is accompanied by certain changes in physical 40 properties of the alloy, such, for example, as increase in density, hardness and tensile strength and decrease in ductility and impact strength. This phase change may occur during 45 the cooling of the alloy after casting or may through certain influences be retarded or inhibited. In such cases it may take place gradually over a period of months at ordinary temperatures.

A secondary stage of phase change which

sometimes occurs is the growth or coalescence of the extremely small particles of the new phases as first formed into larger particles. This stage may be accompanied by softening and lowering of tensile strength and by an 50 increase in ductility and impact strength.

Zinc-aluminum alloys in this range of composition are also subject to a type of disintegration commonly known as intercrystalline oxidation. In extreme cases, under the 55 influence of warmth and moisture, intercrystalline oxidation may completely penetrate specimens of these alloys and cause swelling, warping and even complete disintegration. Intercrystalline oxidation is in some way associated with and partly dependent upon the 60 phase change.

It has heretofore been recognized that certain other metals when present in these zinc-aluminum alloys exercise important effects on either the phase change or the intercrystalline oxidation or both. For example, copper and magnesium are known to exert an influence on the phase change either in respect to the rate at which it takes place or the 65 completeness of the reaction or in some other respect not fully understood. The particular effect produced by copper and magnesium on the phase change reacts favorably in increasing the resistance of the alloys to intercrystalline oxidation. Lead, while not exerting any marked influence on the phase change, very seriously diminishes the resistance of these zinc-aluminum alloys to intercrystalline 70 oxidation. Cadmium, though having a certain effect on the phase change, in the presence of lead also diminishes the resistance of these alloys to intercrystalline oxidation.

Zinc base alloys suitable for die-casting are known and in use. An alloy containing 4% aluminum, 3% copper and the balance high grade zinc metal is widely used and is satisfactory for many purposes. This alloy is, however, open to two objections: First, upon aging, either at normal temperatures 75

or at slightly elevated temperatures, the alloy suffers a serious loss in impact strength and a change in linear dimensions. Second, in the presence of moisture, and particularly in the presence of warmth and moisture together, the alloy undergoes intercrystalline oxidation which causes serious changes in physical properties and dimensions.

An improved zinc base alloy for die-casting is described in the United States patent 10 of Peirce and Anderson, No. 1,596,761, dated August 17, 1926. This alloy (which, as marketed, is usually of the composition 4% aluminum, 3% copper, 0.1% magnesium and 15 the balance high grade zinc) is virtually free from the second fault of the first mentioned alloy, namely, intercrystalline oxidation. It is, however, subject to the first fault, namely, loss of impact strength and change of dimensions upon aging. This objectionable 20 property of these alloys prevents their use in a wide field of otherwise suitable applications. These alloys have a very high tensile strength much beyond that ordinarily needed 25 and the elimination of the faults just described even at the expense of a considerable reduction in tensile strength would be advantageous.

I have discovered that copper (which is 30 present in the foregoing alloys principally to aid in preventing intercrystalline oxidation) is responsible for the loss of impact strength and change in dimensions upon aging, and that an alloy virtually free from 35 objectionable aging changes can be produced from high grade zinc metal by the addition of 4% of aluminum and 0.1% magnesium. This alloy also possesses the other properties requisite in a die-casting alloy. This alloy, 40 when made from high grade zinc metal containing as much as 0.06% of lead plus cadmium, is subject to a certain degree of intercrystalline oxidation which, to some extent, limits its use. I have discovered, however, 45 that by reducing the lead plus cadmium content materially, an alloy of the above composition can be produced which is free from intercrystalline oxidation as well as from aging changes and which will therefore be 50 suitable for a wide range of applications where the two known alloys previously discussed are not satisfactory. Such freedom from intercrystalline oxidation can be secured, for example, by the use of a grade of 55 zinc metal containing 0.01% or less of lead plus cadmium.

Based on these discoveries, my present invention resides in the provision of an improved zinc base die-casting alloy containing 60 an appropriate amount of aluminum for die-casting purposes, say 2 to 15% (preferably about 4%), from 0.01 to 0.3% magnesium (preferably about 0.1%), and the balance high grade zinc metal (preferably 65 containing at least 99.94% zinc). More par-

ticularly, the invention involves the provision of an improved zinc base die-casting alloy containing from 2 to 15% aluminum (preferably not more than 5%), from 0.01 to 0.3% magnesium and in which the zinc 70 base is zinc metal of high purity containing not more than 0.01% of lead plus cadmium and not more than 0.001% tin. In addition, the invention contemplates the provision of a die-casting made of a zinc base alloy and 75 characterized by an impact strength that is not substantially impaired or decreased upon aging at normal or slightly elevated temperatures, and further characterized by a substantially negligible change in linear dimensions upon aging.

It has heretofore been recognized that superior results are usually obtained by employing high grade zinc metal as the zinc base in the known die-casting alloys. The 80 well-known "Horsehead brand" zinc metal has been considered eminently satisfactory for the purpose, and it has not been considered necessary or advantageous to use zinc metal of higher purity. The "Horsehead 85 brand" zinc metal averages 99.94% zinc and contains about 0.045% lead and about 0.003% cadmium.

In its preferred form, the improved zinc 90 base die-casting alloy of the invention is made of a zinc metal base of high purity containing not more than 0.01% lead plus cadmium. Very satisfactory results have been secured with zinc metal containing 99.99+ % zinc, less than 0.003% lead, less than 0.003% 100 cadmium and less than 0.001% tin. Preferably, the zinc base alloy of the invention contains about 4% aluminum, about 0.1% magnesium and the balance zinc metal of high 105 purity containing 99.99+ % zinc. Tin should be substantially excluded from the alloy, and in no case should the tin content exceed about 0.001%.

The following tables illustrate the improved physical properties of die-castings 110 made of the alloy of the invention, more particularly the increase in impact strength (Table II) and the substantially negligible linear expansion (Table III) upon aging. Table IV shows the increase in impact 115 strength and decrease in tensile strength occurring upon simple aging at elevated temperatures (without intercrystalline oxidation or other corrosion). This change is presumably due to some particle growth following the phase change which was presumably completed during the cooling following casting. Alloy A is the preferred composition 120 described in U. S. Patent No. 1,596,761 and alloy D is the preferred composition of the 125 alloy of the present invention. In alloy B the zinc base is zinc metal of high purity instead of high grade zinc metal (Horsehead brand) used in alloy A. In alloy C the zinc base is high-grade zinc metal (Horsehead 130

brand) instead of zinc metal of high purity used in alloy D. In alloys A and C, the zinc metal base contained 99.94+% zinc, while in alloys B and D the zinc metal base contained 99.99+% zinc.

5

*Composition of alloys*

| 10 | Alloy | Al       | Cu       | Mg       | Zinc metal containing— |          |
|----|-------|----------|----------|----------|------------------------|----------|
|    |       |          |          |          | Pb                     | Cd       |
|    |       | Per cent | Per cent | Per cent | Per cent               | Per cent |
| A  |       | 4        | 3        | 0.1      | 0.045                  | 0.003    |
| B  |       | 4        | 3        | 0.1      | 0.0025                 | 0.002    |
| C  |       | 4        | 0        | 0.1      | 0.045                  | 0.003    |
| D  |       | 4        | 0        | 0.1      | 0.0025                 | 0.002    |

*I. Ultimate tensile strength in lbs. per sq. in. (flat tensile specimens)*

| 20 | Alloy  | After exposure to steam at 95° C. |        |        |         |         | After 30 days exposure to steam at 70° C. |
|----|--------|-----------------------------------|--------|--------|---------|---------|-------------------------------------------|
|    |        | As cast                           | 1 day  | 5 days | 10 days | 20 days |                                           |
| A  | 45,100 | 43,600                            | 32,000 | 24,900 | 20,900  | 35,000  |                                           |
| B  | 46,800 | 44,100                            | 43,300 | 43,000 | 38,600  | 42,100  |                                           |
| C  | 37,000 | 37,400                            | 27,900 | 18,800 | 17,100  |         |                                           |
| D  | 41,800 | 36,300                            | 33,600 | 31,900 | 29,400  | 32,800  |                                           |

*II. Impact strength in ft. lbs. per sq. inch*

| 30 | Alloy | After exposure to steam at 95° C. |       |        |         |         | After 30 days exposure to steam at 70° C. |
|----|-------|-----------------------------------|-------|--------|---------|---------|-------------------------------------------|
|    |       | As cast                           | 1 day | 5 days | 10 days | 20 days |                                           |
| A  | 105   | 46                                | 9     | 7      | 6       | 13      |                                           |
| B  | 130   | 94                                | 34    | 17     | 13      | 23      |                                           |
| C  | 109   | 85                                | 20    | 14     |         | 8       |                                           |
| D  | 87    | 109                               | 98    | 95     | 119     |         |                                           |

*III. Linear expansion in inches*

| 40 | Alloy | After exposure to steam at 95° C. |       |        |         |         | After 30 days exposure to steam at 70° C. |
|----|-------|-----------------------------------|-------|--------|---------|---------|-------------------------------------------|
|    |       | As cast                           | 1 day | 5 days | 10 days | 20 days |                                           |
| A  | Width | .7432                             | .0005 | .0033  | .0052   | .0085   | .0027                                     |
| B  |       | .7431                             | .0005 | .0005  | .0019   | .0023   | .0019                                     |
| C  |       | .9814                             | .0000 | .0021  | .0071   |         | .0047                                     |
| D  |       | .7427                             | .0001 | .0003  | .0009   | .0013   | .0007                                     |

*IV. Aging at elevated temperature in dry air*

| 50 | Alloy  | Flat tensile |                   | Impact   |                   | Expansion |
|----|--------|--------------|-------------------|----------|-------------------|-----------|
|    |        | Original     | 10 days at 95° C. | Original | 10 days at 95° C. |           |
| A  | 44,900 | 42,060       |                   | 107      | 21                | 0.0010    |
| D  | 41,800 | 33,700       |                   | 87       | 116               | 0.00000   |

As will be seen from the foregoing tables, the improved alloy of the invention exhibits remarkable retention of its physical properties after accelerated aging. This permits the use of die-castings made of this alloy at elevated temperatures and in the presence of moisture without objectionable impairment of physical properties, and thus permits the

use of such die-castings wherever high grade zinc metal itself is not affected by corroding influences. In addition to the properties illustrated by the tables, die-castings made of the improved alloy of the invention, after accelerated aging for 5 days in steam at 95° C., will withstand a slow bend of about 30° before breaking. Die-castings made of the heretofore available zinc base alloys with which I have worked are capable, after similar aging, of withstanding a slow bend of only about 5° or less. This slow bend test is a measure of the ability of the die-casting to withstand deformation.

I claim:

1. An alloy consisting of 2 to 5% aluminum, 0.01 to 0.3% magnesium and the balance high grade zinc metal.

2. An alloy consisting of approximately 4% aluminum, 0.1% magnesium and the balance high grade zinc.

3. An alloy consisting of 2 to 5% aluminum, 0.01 to 0.3% magnesium and the balance zinc metal containing 99.99% or more zinc.

4. An alloy consisting of 4% aluminum, 0.1% magnesium and the balance zinc metal containing 99.99% or more zinc.

5. A zinc base alloy containing aluminum in sufficient amount to impart satisfactory fluidity to the alloy for die-casting and from 0.01 to 0.3% magnesium and in which the zinc base is zinc metal of high purity containing not more than 0.01% of lead plus cadmium.

6. A zinc base alloy containing from 2 to 15% aluminum, from 0.01 to 0.3% magnesium and in which the zinc base is zinc metal of high purity containing not more than 0.003% lead and not more than 0.003% cadmium and not more than 0.001% tin.

7. A zinc base alloy containing from 2 to 15% aluminum, from 0.01 to 0.3% magnesium and in which the zinc base is zinc metal containing 99.99% zinc and less than 0.01% of lead plus cadmium.

8. A zinc base alloy containing about 4% aluminum, about 0.1% magnesium and in which the zinc base is zinc metal of high purity containing not more than 0.01% of lead plus cadmium.

9. A zinc base alloy containing about 4% aluminum, about 0.1% magnesium and in which the zinc base is zinc metal containing 99.99+% zinc and not more than 0.003% lead and not more than 0.003% cadmium and not more than 0.001% tin.

10. A zinc base alloy containing about 4% aluminum, about 0.1% magnesium and in which the zinc base is zinc metal containing 99.99+% zinc and less than 0.01% of lead plus cadmium.

In testimony whereof I affix my signature.

EDMUND A. ANDERSON.

70

75

80

85

90

95

100

105

110

115

120

125

130